



US008327917B2

(12) **United States Patent**  
**Sato**

(10) **Patent No.:** **US 8,327,917 B2**  
(b4) **Date of Patent:** **Dec. 11, 2012**

(54) **APPARATUS FOR PRODUCING  
AMORPHOUS ALLOY FOIL STRIP AND  
METHOD FOR PRODUCING AMORPHOUS  
ALLOY FOIL STRIP**

(75) Inventor: **Takashi Sato**, Kanagawa-ken (JP)

(73) Assignee: **Nippon Steel Corporation**, Tokyo (JP)

(\*) Notice: Subject to any disclaimer, the term of this patent is extended or adjusted under 35 U.S.C. 154(b) by 0 days.

(21) Appl. No.: **12/919,043**

(22) PCT Filed: **Feb. 20, 2009**

(86) PCT No.: **PCT/JP2009/053067**

§ 371 (c)(1),  
(2), (4) Date: **Oct. 29, 2010**

(87) PCT Pub. No.: **WO2009/107561**

PCT Pub. Date: **Sep. 3, 2009**

(65) **Prior Publication Data**

US 2011/0036532 A1 Feb. 17, 2011

(30) **Foreign Application Priority Data**

Feb. 25, 2008 (JP) ..... 2008-042696  
Oct. 22, 2008 (JP) ..... 2008-272421  
Oct. 22, 2008 (JP) ..... 2008-272422

(51) **Int. Cl.**

**B22D 11/06** (2006.01)  
**B22D 27/04** (2006.01)

(52) **U.S. Cl.** ..... **164/428; 164/136; 164/423; 164/438;  
164/463; 164/480**

(58) **Field of Classification Search** ..... **164/463,  
164/480, 137, 337, 423, 136, 428**

See application file for complete search history.

(56)

**References Cited**

**U.S. PATENT DOCUMENTS**

4,428,416 A \* 1/1984 Shimanuki et al. ..... 164/461  
4,546,815 A \* 10/1985 Liebermann et al. ..... 164/463  
4,600,048 A \* 7/1986 Sato et al. ..... 164/463

(Continued)

**FOREIGN PATENT DOCUMENTS**

JP 59-064144 A 4/1984

(Continued)

**OTHER PUBLICATIONS**

International Search Report for PCT/JP2009/053067 dated Apr. 28, 2009.

(Continued)

*Primary Examiner* — Devang R Patel

(74) *Attorney, Agent, or Firm* — Pearne & Gordon LLP

(57)

**ABSTRACT**

An apparatus and a method for producing an amorphous alloy foil strip, which are capable of producing an amorphous alloy foil strip having a large sheet thickness in an industrial scale, are provided.

A production apparatus **101** for an amorphous alloy foil strip **S** includes: a pair of cooling rolls **113a** and **113b**; a driving unit **111** configured to rotate the cooling rolls; and a crucible **114** configured to supply a molten alloy sequentially to an outer circumferential surface of the cooling roll **113a** and an outer circumferential surface of the cooling roll **113b**. The crucible **114** is movable along a moving unit **116**. A molten alloy is supplied alternately to the cooling roll **113a** and the cooling roll **113b** while rotating and water-cooling the cooling rolls **113a** and **113b**.

**7 Claims, 18 Drawing Sheets**



U.S. PATENT DOCUMENTS

4,650,618 A \* 3/1987 Heinemann et al. .... 264/431  
4,676,298 A \* 6/1987 Liebermann ..... 164/463  
6,755,234 B2 \* 6/2004 Blejde et al. ..... 164/151.4

JP 06-086847 A 3/1994  
JP 07-310149 A 11/1995  
JP 10-085910 A 4/1998  
JP 2002-283010 A 10/2002

FOREIGN PATENT DOCUMENTS

JP 60-108144 A 6/1985  
JP 61199554 A \* 9/1986  
JP 61-59817 A 12/1986  
JP 64-005945 A 1/1989

OTHER PUBLICATIONS

Chinese Office action for 200980106060.9 dated Jul. 4, 2012.  
Taiwanese Office action for 98105756 dated Jul. 20, 2012.

\* cited by examiner



FIG. 1



FIG. 2



FIG. 3



FIG. 4



FIG. 5



FIG. 6A

FIG. 6B

FIG. 6C

FIG. 7A



FIG. 7B



TIME →  
(UPSTREAM → DOWNSTREAM)  
(PUDDLE → DETACHMENT)



FIG. 8



FIG. 9A



FIG. 9B



FIG. 10



FIG. 11



FIG. 12A



FIG. 12B



FIG. 13



FIG. 14



FIG. 15



FIG. 16



FIG. 17



FIG. 18



FIG. 19



FIG. 20



FIG. 21



FIG. 22

## 1

**APPARATUS FOR PRODUCING  
AMORPHOUS ALLOY FOIL STRIP AND  
METHOD FOR PRODUCING AMORPHOUS  
ALLOY FOIL STRIP**

TECHNICAL FIELD

The invention relates to an apparatus for producing an amorphous alloy foil strip and a method for producing an amorphous alloy foil strip, and more specifically, to an apparatus for producing an amorphous alloy foil strip provided with cooling rolls and a method for producing an amorphous alloy foil strip.

BACKGROUND ART

Use of an iron-base amorphous alloy having less power loss as an iron core of a transformer or a motor has heretofore been studied and has been put into practice in some transformers. However, the amorphous alloy has not been practically used in motors and is used only for wound iron cores even in transformers. This is because the sheet thicknesses of amorphous alloy foil strips produced in an industrial scale are as extremely thin as 25  $\mu\text{m}$  or below. If thick foil strips are produced industrially, the amorphous alloy can be also used in motors and in stacked iron-core transformers. An increase in the thickness of foil strips improves operation efficiency of iron-core production processes and also enhances a space factor. Moreover, mechanical strength of an iron core is significantly enhanced by improving rigidity of the foil strips. In other words, the amorphous alloy can be used for a motor provided with an iron core formed by stacking the foil strips or for a stacked iron core.

The most common method for producing an amorphous alloy is a roll liquid quenching method including quenching and solidifying a molten alloy into a foil strip shape by bringing the molten alloy into contact with an outer circumferential surface of a roll, made of metal or an alloy having high thermal conductivity, while rapidly rotating the roll. However, there is a stringent restriction of the sheet thickness of the amorphous alloy foil strip that can be produced by the roll liquid quenching method and it has therefore not been possible to produce a sufficiently thick foil strip.

To address this issue, the inventors of the invention have developed a multiple-slit nozzle method using multiple slits arranged in a circumferential direction of a roll, and have disclosed the method in Patent Document 1. According to this multiple-slit nozzle method, a molten alloy ejected from the slits forms multiple puddles in a small space between the nozzle and the roll, the number of puddles corresponding to the number of the slits. A first puddle, counted from an upstream, around a contact surface thereof with the roll is cooled down on an outer circumferential surface of the roll, whereby a supercooled fluid layer with increased viscosity is drawn by the roll and a puddle on a downstream side is superimposed thereon. The temperature of the fluid layer drawn from the upstream puddle is lowered before the fluid layer meets the downstream puddle. Accordingly, the downstream puddle is cooled down by this fluid layer and a portion with increased viscosity is drawn out. A thick foil strip is formed by repeating this operation. As the fluid layers are superimposed on one another in a liquid state, interfaces thereof are mixed together so that an integrated amorphous alloy foil strip without interlayer boundaries can be obtained.

However, even the multiple-slit nozzle method has the following problem. Specifically, the roll liquid quenching method includes a method using a non-water-cooled roll and

## 2

a method using a water-cooled roll. The non-water-cooled roll cools the molten alloy down by a heat capacity of the roll itself. In the case of using the non-water-cooled roll, it is possible to cool the molten alloy down efficiently and to produce a certain amount of thick amorphous alloy foil strip at an initial producing state when the roll temperature is low. However, the non-water-cooled roll reduces cooling efficiency when the roll temperature is increased and therefore cannot be used for a long period of time. Accordingly, this is not suitable to produce the amorphous alloy foil strips industrially.

Due to this reason, it is preferable to use the water-cooled roll from an industrial perspective. As a water cooling mechanism is embedded in the water-cooled roll, it is possible to radiate the heat by way of cooling water even when the roll itself has a small heat capacity. However, the thick amorphous alloy having a sheet thickness exceeding 25  $\mu\text{m}$  has been difficult to mass-produce in an industrial scale even by using the water-cooled roll.

20 [Patent Document 1] JP S60-108144 A

[Patent Document 2] JP H6-86847 U

[Patent Document 3] JP S61-059817 B

DISCLOSURE OF THE INVENTION

25 [Problems to be Resolved by the Invention]

The purpose of the invention is to provide an apparatus for producing an amorphous alloy foil strip and a method for producing an amorphous alloy foil strip, which are capable of producing an amorphous alloy foil strip having a large sheet thickness in an industrial scale.

30 [Means for Solving the Problems]

According to an aspect of the invention, there is provided an apparatus for producing an amorphous alloy foil strip, including: a first cooling roll; a second cooling roll; a driving unit configured to rotate the first and second cooling rolls; and a supply unit configured to supply a molten alloy sequentially to an outer circumferential surface of the first cooling roll and an outer circumferential surface of the second cooling roll.

35 40 According to another aspect of the invention, there is provided an apparatus for producing an amorphous alloy foil strip, including: a cooling roll; a driving unit configured to rotate the cooling roll; and a supply unit configured to supply a molten alloy to an outer circumferential surface of the cooling roll, the cooling roll including: first and second cooling zones surrounding an outer circumferential portion of the cooling roll and being separated from each other in an axial direction of the cooling roll; and a heat insulating zone disposed between the first cooling zone and the second cooling

45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9

a first cooling zone while rotating a cooling roll, the first cooling zone being provided surrounding an outer circumferential portion of the cooling roll; and a second process of supplying the molten alloy to a second cooling zone while rotating the cooling roll, the second cooling zone being provided surrounding the outer circumferential portion of the cooling roll and located away from the first cooling zone in an axial direction of the cooling roll, the first process and the second process being alternately executed.

According to yet another aspect of the invention, there is provided a method for producing an amorphous alloy foil strip, including: a first process of supplying a molten alloy to a first cooling zone while rotating a cooling roll, the first cooling zone being provided surrounding an outer circumferential portion of the cooling roll; and a second process of supplying the molten alloy to a second cooling zone while rotating the cooling roll, the second cooling zone being provided surrounding the outer circumferential portion of the cooling roll and located away from the first cooling zone in an axial direction of the cooling roll with a heat insulating zone interposed between the first cooling zone and the second cooling zone, the heat insulating zone being made of a material having lower thermal conductivity than a material used for forming the first cooling zone, the second cooling zone being made of a material having higher thermal conductivity than the material used for forming the heat insulating zone, the first process and the second process being alternately executed.

According to yet another aspect of the invention, there is provided a method for producing an amorphous alloy foil strip, including: a first process of supplying a molten alloy to a first cooling zone while rotating a cooling roll, the first cooling zone forming part of an outer circumferential portion of the cooling roll and extending along a circumferential direction of the cooling roll; and a second process of supplying the molten alloy to a second cooling zone while rotating the cooling roll, the second cooling zone being separated from the first cooling zone in an axial direction of the cooling roll with a forbidden zone interposed between the first cooling zone and the second cooling zone, and extending along the circumferential direction of the cooling roll, the first process and the second process being alternately executed.

#### [Effects of the Invention]

According to the invention, an apparatus for producing an amorphous alloy foil strip and a method for producing an amorphous alloy foil strip, which are capable of producing an amorphous alloy foil strip having a large sheet thickness in an industrial scale, can be realized.

#### BRIEF DESCRIPTION OF DRAWINGS

FIG. 1 is a front view illustrating a production apparatus for an amorphous alloy foil strip according to a first embodiment of the invention.

FIG. 2 is a cross-sectional view illustrating a portion where a molten alloy comes in contact with a cooling roll in FIG. 1.

FIG. 3 is a conceptual diagram illustrating a pathway of cooling water circulated in the cooling roll in FIG. 1.

FIG. 4 is a timing chart illustrating a method for producing an amorphous alloy foil strip according to the first embodiment, in which a horizontal axis indicates time and a vertical axis indicates cooling rolls.

FIG. 5 is a ternary composition diagram illustrating a composition of an iron-base amorphous alloy foil strip to be produced in the embodiment.

FIGS. 6A to 6C are explanatory diagrams defining the wall thickness of the cooling roll in the embodiment.

FIG. 7A schematically shows the time change of the temperature of a foil strip in the course of casting, and FIG. 7B schematically shows the temperature change of the surface of the cooling zone.

FIG. 8 is a schematic view comparing the time change of the temperature of the roll surface in the course of casting a thick foil strip between (a) the case of using a roll having a small wall thickness and (b) the case of using a roll having a large wall thickness.

FIGS. 9A and 9B are schematic views illustrating the temperature change of a thick wall direction of the cooling roll in the course of casting an amorphous alloy foil strip, in which (a) shows the thin wall roll and (b) shows the thick wall roll.

FIG. 10 is a perspective view illustrating a production apparatus for an amorphous alloy foil strip according to a second embodiment of the invention.

FIG. 11 is a cross-sectional view illustrating the vicinity of a cooling roll shown in FIG. 10.

FIGS. 12A and 12B are cross-sectional views illustrating a cooling roll in a variation 1 of the second embodiment, in which FIG. 12A shows a branch pipe including a valve and FIG. 12B shows a roll including a fin.

FIG. 13 is a cross-sectional view of the vicinity of a cooling roll in a production apparatus for an amorphous alloy foil strip according to a variation 2 of the second embodiment.

FIG. 14 is a front view illustrating a production apparatus for an amorphous alloy foil strip according to a third embodiment of the invention.

FIG. 15 is a cross-sectional view illustrating the structure of a cooling roll of FIG. 14.

FIG. 16 is a conceptual diagram illustrating a pathway of cooling water to cool the cooling roll in FIG. 14.

FIG. 17 is a timing chart illustrating a method for producing an amorphous alloy foil strip according to the embodiment, in which a horizontal axis indicates time and a vertical axis indicates cooling zones.

FIG. 18 is a cross-sectional view of a water channel illustrating a fin provided in the inner surface in contact with cooling water of a cooling zone.

FIG. 19 is a front view illustrating a production apparatus for an amorphous alloy foil strip according to a fourth embodiment of the invention.

FIG. 20 is a cross-sectional view illustrating the structure of a cooling roll of FIG. 19.

FIG. 21 is a conceptual diagram illustrating a pathway of cooling water circulated in the cooling roll in FIG. 19.

FIG. 22 is a graph illustrating influences of the width of a forbidden zone on the sheet thickness deviation of an amorphous foil strip.

#### EXPLANATION OF REFERENCE

|    |                                                                                                                                                                                                            |                                                                                                                                                                                                                                                      |
|----|------------------------------------------------------------------------------------------------------------------------------------------------------------------------------------------------------------|------------------------------------------------------------------------------------------------------------------------------------------------------------------------------------------------------------------------------------------------------|
| 55 | 101, 102, 103, 201, 301<br>111, 211, 311<br>112a, 112b, 212a, 212b, 312a, 312b<br>113a, 113b, 213, 313<br>114, 214, 314<br>115, 215, 315<br>116, 216, 316<br>117a, 117b<br>119<br>120<br>121<br>122<br>123 | production apparatus<br>driving unit<br>rotating shaft member<br>cooling roll<br>crucible<br>nozzle<br>moving unit<br>slit<br>open roll side surface<br>opening<br>inner circumferential surface<br>partition plate<br>side surface<br>water channel |
| 60 | 124, 224, 324                                                                                                                                                                                              |                                                                                                                                                                                                                                                      |
| 65 |                                                                                                                                                                                                            |                                                                                                                                                                                                                                                      |

|                                         |                      |
|-----------------------------------------|----------------------|
| 125, 225, 325                           | feed pipe            |
| 125a                                    | branch pipe          |
| 126, 226, 326                           | drain pipe           |
| 126a                                    | branch pipe          |
| 127                                     | partition plate      |
| 128, 228                                | fin                  |
| 133                                     | cooling roll         |
| 134                                     | through hole         |
| 135                                     | convex portion       |
| 136                                     | flange               |
| 137                                     | drain outlet         |
| 138                                     | entrance portion     |
| 139                                     | water supply pipe    |
| 141, 141a, 141b, 241a, 241b, 341a, 341b | bearing              |
| 142, 242, 342                           | water tank           |
| 143, 243, 343                           | cooling unit         |
| 144                                     | valve                |
| 213a, 213b, 313a, 313b                  | cooling zone         |
| 218                                     | heat insulating zone |
| 231, 331                                | supporting mechanism |
| 232, 332                                | central part         |
| 318                                     | forbidden zone       |
| A                                       | molten alloy         |
| P                                       | puddle               |
| R                                       | Region               |
| S                                       | foil strip           |
| W                                       | cooling water        |

## Best Modes for Carrying out the Invention

Hereinafter, embodiments of the invention will be described with reference to the drawings.

First of all, a first embodiment of the invention will be described.

FIG. 1 is a front view illustrating a production apparatus for an amorphous alloy foil strip according to this embodiment. FIG. 2 is a cross-sectional view illustrating a portion where a molten alloy comes in contact with a cooling roll in FIG. 1. FIG. 3 is a conceptual diagram showing a pathway of cooling water circulated in the cooling roll in FIG. 1.

As shown in FIG. 1, a production apparatus 101 for an amorphous alloy foil strip according to this embodiment is configured to mainly produce an iron-base amorphous alloy foil strip (hereinafter also simply referred to as a "foil strip") S. The production apparatus 101 includes two cooling rolls 113a and 113b (hereinafter also collectively referred to as "cooling rolls 113") which are located in both sides of a driving unit 111. The cooling rolls 113a and 113b are rotatably supported by rotating shaft members 112a and 112b, respectively. A motor (not shown) is embedded in the driving unit 111 and is configured to rotate the cooling rolls 113 via a pair of the rotating shaft members 112a and 112b. The rotating shaft members 112 and the cooling rolls 113 are supported by bearings 141, 141a, and 141b. The cooling rolls 113a and 113b are made of metal or an alloy having high thermal conductivity, and are made of, for example, copper or a copper alloy.

The production apparatus 101 is provided with a crucible 114 for retaining a molten alloy A (see FIG. 2), and a nozzle 115 for ejecting the molten alloy A in the crucible 114 to outside of the crucible 114 is fitted to a lower end of the crucible 114. Here, the crucible is not limited to the one shown in FIG. 1 and includes all measures for storing and supplying molten metal. For example, a device capable of receiving the molten metal from an alloy melter and supplying the alloy to the cooling roll through a nozzle will be called the crucible. An apparatus configured to provide a melter with a nozzle and capable of directly supplying the molten metal is also included in the crucible.

Further, the production apparatus 101 is provided with a moving unit 116 extending in a direction from the cooling roll

113a toward the cooling roll 113b. Accordingly, the crucible 114 is guided by the moving unit 116 and is movable between a position where the molten alloy A can be ejected from a perpendicular direction relative to an outer circumferential surface of the cooling roll 113a, and a position where the molten alloy A can be ejected from a perpendicular direction relative to an outer circumferential surface of the cooling roll 113b. An ejection port of the nozzle 115, that is, a slit is oriented in the perpendicular direction relative to the outer circumferential surfaces of the rolls and a slight clearance is maintained with the outer circumferential surface of the cooling roll 113a or 113b. The crucible 114, the nozzle 115, and the moving unit 116 constitute a supplying unit for the molten alloy A.

15 As shown in FIG. 2, the nozzle 115 is a multiple-slit nozzle. Specifically, the shape of the ejection port of the nozzle 115 is formed into a shape in which multiple slits, e.g., two slits 117a and 117b, are arranged along a circumferential direction of the cooling rolls 113. The longitudinal direction of each of 20 the slits 117a and 117b is identical to an axial direction (a roll width direction) of the cooling rolls 113. The distance between the slits 117a and 117b is, for example, set equal to or below 10 mm (millimeters), and is, for example, equal to or below 6 mm. Here, a multiple-slit nozzle including three or 25 more slits formed at the ejection port or a single-slit nozzle provided with only one slit may be used as the nozzle 115.

The nozzle 115 is made of a refractory material which is less wettable to the molten alloy A, and is made of boron nitride, zirconia or alumina, for example. In this way, the slits 30 are prevented from being clogged with the molten alloy A, i.e., configured to eject it smoothly. Besides these refractory materials, a refractory material that allows permeation of the molten alloy can be used as the material of the nozzle 115 if a surface thereof is coated with a substance which is less 35 wettable to the molten alloy by thermal spray or the like. For example, silicon nitride or the like has excellent strength and thermal shock. A composite material of silicon carbide and boron carbide has electric conductivity in addition to heat resistance and facilitates heat retention of the nozzle in a 40 standby state. However, these materials react with iron inside the molten alloy and therefore need to be coated with the above-described less wettable material such as boron nitride, zirconia or alumina.

FIG. 3 shows a simplified pathway of cooling water W in 45 the production apparatus 101. In FIG. 3, the cooling water W for cooling down the cooling roll 113 is supplied using a pump (not shown) from a water tank 142 to a water channel 124 inside the cooling rolls via a feed pipe 125, and after circulation in the water channel 124, is returned to the water 50 tank via a drain pipe 126. In order to retain the cooling water lower than a predetermined temperature such as a room temperature during casting, a cooling unit 143 configured to cool the cooling water W down is provided in the course of the pathway of the cooling water W, e.g., in the water tank 142. 55 The cooling unit 143 may be a unit applying a heat pump, a unit for feeding a material such as ice which has a lower temperature than the room temperature, and so forth.

Next, operations of the production apparatus 101 according to this embodiment configured as described above, that is, a method for producing an amorphous alloy foil strip according to this embodiment will be described.

First, as shown in FIG. 1, the cooling rolls 113a and 113b are rotated by way of the rotating shaft members 112a and 112b by driving the driving unit 111. Next, the molten alloy A 60 is ejected from the crucible 114 to the outer circumferential surface of one of the cooling rolls 113a through the nozzle 115 which is closely located at a predetermined interval. In

this way, a puddle P is formed between the nozzle 115 and the cooling roll 113a. Then, a portion of the molten alloy forming the puddle P, which contacts the cooling roll, is cooled down so as to increase viscosity and is drawn out of the puddle P by rotation of the cooling roll 113a. The alloy thus drawn out is a supercooled liquid at this point, but is quenched by the roll down to a glass transition temperature or below and is formed into the amorphous alloy foil strip S. A cooling rate required for rendering the foil strip (or the supercooled liquid) drawn out of the puddle amorphous is equal to or above  $1 \times 10^5$ ° C./sec. in the case of the iron-base alloy, for example.

In this embodiment, two slits 117 are formed in the nozzle 115 as shown in FIG. 2. For this reason, the sheet thickness of the formed foil strip becomes thicker than the case of using a single slit even if a circumferential velocity of the cooling roll is the same. That is, productivity is high. The sheet thickness with the multiple-slit nozzle is thicker than that with the single-slit nozzle under the condition of the same roll circumferential velocity. This is because a contact area with a cooling zone is increased by splitting the puddles P into multiple portions, and thereby a heat flow to be transmitted to the cooling zone can be dispersed.

The heat transmitted from the molten alloy and the foil strip to the cooling roll 113a in order to form the amorphous alloy foil strip is transferred from the outer circumferential portion of the cooling roll 113a inward and transmitted to the cooling water W circulated inside the water channel. That is, the heat of the molten alloy A is discharged by way of the molten alloy A→the cooling roll 113a→the cooling water W.

When the temperature of the cooling roll 113a reaches a predetermined value along with casting of the foil strip S, the nozzle 115 is closed to stop ejection of the molten alloy A. Next, the crucible 114 is moved along a rail of the moving unit 116 and the nozzle 115 is disposed close to the outer circumferential surface of the other cooling roll 113b. Subsequently, the nozzle 115 is opened again to eject the molten alloy A toward the outer circumferential surface of the cooling roll 113b. In this way, a foil strip S is cast with the cooling roll 113b by the same operation as the operation with the cooling roll 113a. In other words, as shown in FIG. 4, the cooling roll used for casting the foil strips S is switched from the cooling roll 113a to the cooling roll 113b. Although the cooling roll 113a is in a standby state in this period, the cooling water W is continuously supplied to the cooling roll 113a as well to cool the cooling roll 113a down.

Further, when the temperature of the cooling roll 113b reaches the predetermined value, the cooling roll used for casting the foil strips S is switched from the cooling roll 113b to the cooling roll 113a. By this time, the cooling roll 113a is cooled down to the temperature before casting so that it is possible to resume casting the foil strip S. Here, the cooling water W is continuously supplied to the cooling roll 113b in the standby state as well in this period to continue cooling. Likewise, as shown in FIG. 4, the cooling roll 113a and the cooling roll 113b are alternately used thereafter to continue production of the foil strips S.

In this way, it is possible to continue production of the foil strips S always by use of the cooling rolls at the temperature equal to or below the predetermined value by alternating the processes of supplying the molten alloy A to the outer circumferential surface of the cooling roll 113a while rotating the cooling roll 113a and cooling the cooling roll 113a down without supplying the molten alloy A to the outer circumferential surface of the cooling roll 113b.

Examples of numerical values in this embodiment will now be shown below.

FIG. 5 is a ternary composition diagram illustrating a composition of the iron-base amorphous alloy foil strip to be produced in this embodiment. The iron-base amorphous alloy foil strip S to be produced in this embodiment has a width, for example, equal to or above 60 mm and a thickness (a sheet thickness), for example, equal to or above 30  $\mu\text{m}$  (micrometers), e.g., equal to or above 33  $\mu\text{m}$ , and, e.g., equal to or above 40  $\mu\text{m}$ . Here, in this specification, the thickness of the foil strip is defined by use of a weight sheet thickness. The weight sheet thickness is a value obtained by dividing the weight of the foil strip by the area and the density of the foil strip.

As shown in FIG. 5, the composition of this iron-base amorphous alloy foil strip S is achieved by adding, for example, metalloids, i.e., silicon (Si) and boron (B), to iron (Fe). When using this foil strip S for an electromagnetic application, it is preferable to set the concentration of iron equal to or above 70 at %. For example, the composition of the foil strip is set to a concentration located in a region R surrounded by a dashed line in FIG. 5, i.e., the content of iron in a range from 70 to 81 at %, the content of silicon in a range from 3 to 17 at %, the content of boron in a range from 9 to 23 at %, and a glass transition temperature  $T_g$  equal to or above 500° C. Here, a sum of iron, silicon, boron, and unavoidable impurities is equal to 100 at %. Here, part of iron may be replaced by cobalt (Co) or nickel (Ni). The amount of replacement is set equal to or below 20 at % in total. Also, part of silicon or boron may be replaced by carbon which is equal to or below 2.0 at %. It is to be noted, however, that the amount of replacement by carbon is set within the range where the glass transition temperature  $T_g$  is equal to or above 500° C. In other words, the composition of the molten alloy A may be set to the composition in which the content of iron is set in a range from 70 to 81 at %, the content of silicon is set in a range from 1 to 17 at %, the content of boron is set in a range from 7 to 23 at %, the content of carbon is set equal to or below 2 at %, and the glass transition temperature  $T_g$  is set equal to or above 500° C.

The reason for defining the glass transition temperature  $T_g$  as the prerequisite for selecting the composition is as follows. Previously, ease of forming an amorphous alloy (glass forming ability) has been evaluated by a ratio ( $T_g/T_m$ ) between the melting point  $T_m$  of the alloy and the glass transition temperature  $T_g$  (which is the absolute temperature in this case). However, in reality, the glass transition temperature  $T_g$  exhibits more significant contribution than the melting point  $T_m$  and the region R of the alloy composition is therefore defined by the magnitude of  $T_g$ . When the glass transition temperature  $T_g$  of the alloy is raised by 50° C., the upper limit sheet thickness of the foil strip that can be amorphous is increased at least by 10%. Here, it is difficult to measure the glass transition temperature  $T_g$  in the case of an iron-base alloy. Accordingly, a crystallization peak temperature  $T_{p1}$  that is deemed to be almost the same temperature is used instead. The numerical values in FIG. 5 represent the crystallization peak temperatures  $T_{p1}$  (° C.).

Of the compositions in the region R shown in FIG. 5, concrete compositions of groups having relatively high saturation magnetic flux densities  $B_s$ , i.e., the groups having the saturation magnetic flux densities  $B_s$  equal to or above 1.5 T (tesla), and of groups having low hysteresis losses are respectively shown in Table 1. The hysteresis loss is a hysteresis loss  $W_{h13/50}$  at a frequency of 50 Hz (hertz) and at a magnetic flux density of 1.3 T. In Table 1, the value  $W_{h13/50}$  of any of the compositions shown in the right column is equal to or below 0.08 W/kg when performing a heat treatment under optimum conditions. Here, the hysteresis loss  $W_{h13/50}$  is the value

measured by use of a single-sheet sample. Here, numbers indicated in Table 1 represent atomic percentage of the respective components.

TABLE 1

| Examples of Compositions Having High Saturation Magnetic Flux Densities | Examples of Compositions Having Low Hysteresis Losses |
|-------------------------------------------------------------------------|-------------------------------------------------------|
| Fe <sub>81</sub> Si <sub>6</sub> B <sub>13</sub>                        | Fe <sub>75</sub> Si <sub>10</sub> B <sub>15</sub>     |
| Fe <sub>80</sub> Si <sub>6</sub> B <sub>14</sub>                        | Fe <sub>74</sub> Si <sub>12</sub> B <sub>14</sub>     |
| Fe <sub>79</sub> Si <sub>6</sub> B <sub>15</sub>                        | Fe <sub>73</sub> Si <sub>11</sub> B <sub>16</sub>     |
| Fe <sub>78</sub> Si <sub>6</sub> B <sub>16</sub>                        |                                                       |
| Fe <sub>77</sub> Si <sub>10</sub> B <sub>13</sub>                       |                                                       |
| Fe <sub>76</sub> Si <sub>10</sub> B <sub>14</sub>                       |                                                       |
| Fe <sub>76</sub> Si <sub>10</sub> B <sub>16</sub>                       |                                                       |

The foil strip S may also contain in (Sn) in a range from 0.01 to 1.0 mass %. While crystallization of the foil strip is initiated from a surface thereof, it has a strong tendency to be segregated on the surface and exhibits an effect to suppress crystallization of a foil strip surface layer. In this way, deterioration in a magnetic characteristic associated with crystallization is suppressed. Moreover, it has an effect to suppress a variation of the magnetic characteristic with time.

Next, the production apparatus and the production method according to this embodiment will be described in detail.

The cooling roll 113 preferably has a wall thickness equal to or above 25 mm. Here, as shown in FIGS. 6A to 6C, the wall thickness of the cooling roll 113 is equivalent to a distance from the outer circumferential surface of the cooling roll to an inner surface of the cooling roll contacting the cooling water. When a cross section orthogonal to the water channel 124 has a shape of a circular pipe, for example, a distance from a portion closest to the outer circumferential surface to the outer circumferential surface is defined as the wall thickness 129 of the cooling roll as shown in FIG. 6A. If the cross section of the water channel has any of a rectangular shape and a rectangular shape provided with fins 128, then distances shown in FIGS. 6B and 6C are respectively defined as the wall thickness 129 of the cooling roll.

Previously, the wall thickness of the cooling roll has been designed on the premise of continuous casting for a long time period. The thinner wall surface has been deemed to be more advantageous in light of heat discharge and a thickness equal to or below 10 mm has been adopted. For example, Patent Document 2 defines the wall thickness of a cooling roll (a cooling sleeve) in a range from 3 to 10 mm and describes the reason. According to the document, when the thickness exceeds 10 mm, there is a large drop in a cooling rate that intensifies local embrittlement of an amorphous alloy foil strip, and in particular, it is not possible to obtain a foil strip having a sheet thickness equal to or above 25  $\mu$ m which can be bent fully. On the other hand, the thickness equal to or below 3 mm causes large thermal deformation of the cooling roll that leads to an uneven thickness of a quenched foil strip. Moreover, Patent Document 2 discloses a method of causing a jet of cooling water to run into an inner surface of a roll as a unit for thickening an amorphous alloy foil strip. However, this method still has a limited effect to increase a heat transfer coefficient between the roll and the water and therefore faces a difficulty in producing an amorphous alloy foil strip having a sheet thickness exceeding 30  $\mu$ m.

The reason why it is difficult to obtain a thick amorphous alloy foil strip by using the conventional cooling roll having a thin wall thickness will be described based on experimental knowledge and heat transfer calculation. FIG. 7A schematically shows the time change (corresponding to a distance in

downstream direction from the puddle) of the temperature of a foil strip in the course of casting (including an unsolidified fluid) and FIG. 7B schematically shows the temperature change of the surface of the cooling roll. Concerning respective curved lines in the drawing, a line (1) indicates a case of producing a thin foil strip (e.g., 25  $\mu$ m) by using a cooling roll having a small wall thickness (the conventional method, e.g., 10 mm), a line (2) indicates a case of producing a thick foil strip (e.g., 40  $\mu$ m) by using the cooling roll having a small wall thickness (the conventional method, e.g., 10 mm), and a line (3) indicates a case of producing the thick foil strip (e.g., 40  $\mu$ m) by using a cooling roll having a large wall thickness (this embodiment, e.g., 30 mm).

As shown in FIG. 7A, the curved line (1) indicating the temperature change of the foil strip represents the case of producing the thin foil strip by use of the roll having a small wall thickness, in which time  $t_1$  lapsed from the melting point  $T_m$  of the alloy to the glass transition temperature  $T_g$  is sufficiently shorter than critical time for vitrification  $t_g$  and the foil strip is cooled down at a cooling rate that is necessary for forming the amorphous body. On the other hand, the line (2) represents the case of producing the thick foil strip by use of the same roll having a small wall thickness, in which a gradient of the temperature curve is reduced as compared to the gradient of the line (1) when the line comes close to the glass transition temperature  $T_g$ . Accordingly, time  $t_2$  lapsed from  $T_m$  to  $T_g$  becomes longer than  $t_g$ . That is, it is not possible to obtain the cooling rate necessary for forming the amorphous body.

On the other hand, the cooling curve in the case of producing the thick foil strip by use of the cooling roll having a thick cooling zone as in this embodiment is formed into the line (3), which has reduction in the gradient in the vicinity of the glass transition temperature  $T_g$  smaller than the condition of the line (2). Accordingly, the time  $t_2$  to reach  $T_g$  becomes shorter than  $t_g$  and the foil strip is cooled down at the cooling rate necessary for forming the amorphous body, thereby forming the thick amorphous alloy foil strip.

The sheet thickness of the amorphous alloy foil strip, which is intended to be produced, constitutes a basis for designing the wall thickness of the cooling roll. The wall thickness of the cooling roll 113 is increased depending on the sheet thickness of the foil strip. It is preferable to set the wall thickness of the cooling roll 113 equal to or above 25 mm in order to form the thick foil strip having a sheet thickness equal to or above 30  $\mu$ m. For example, the wall thickness of the cooling roll 113 is set equal to 30 mm when the sheet thickness of the foil strip S is in a range from 30 to 45  $\mu$ m. The wall thickness of the cooling roll is set equal to 50 mm when the sheet thickness of the foil strip S is in a range from 45 to 60  $\mu$ m. The wall thickness of the cooling roll is set equal to 100 mm when the sheet thickness of the foil strip S is in a range from 60 to 120  $\mu$ m.

In this embodiment, the circumferential velocity of the cooling roll is set in a range from 10 to 30 m/sec., for example, 20 m/sec. In an alternate casting method using twin rolls as in this embodiment, timing for change is set up depending on the surface temperatures of the cooling rolls 113, for example. When the temperature on a puddle upstream side of the cooling roll 113a reaches 200° C., for example, the cooling roll used for casting is changed to the cooling roll 113b. At this time, a measurement position for the temperature of the cooling roll is defined in a position located 20 cm away on an upstream side from the nozzle 115, for example. Alternatively, if the sheet thickness, the width, and casting conditions of the foil strip S are constant, it is also possible to change based on a numerical value measured in advance.

When producing the amorphous alloy foil strips only by use of a single cooling roll as in the conventional case, it is extremely difficult to continuously produce the foil strips having a sheet thickness larger than 30  $\mu\text{m}$ . No matter how favorably the shape, the size, and a cooling mechanism of the cooling roll are designed within practical ranges, the temperature of the outer circumferential surface of the cooling roll continues to rise along with casting time. Then, if the temperature of the outer circumferential surface of the cooling roll rises above the aforementioned critical temperature (e.g., 200° C.), the cooling rate necessary for forming the amorphous body becomes unavailable and the foil strips begin to crystallize.

Description will be made by use of FIG. 8 in order to help understanding the above-described heat transfer behavior. FIG. 8 schematically shows transition of the temperature of the outer circumferential surface of the cooling roll when producing (a) the thick foil strip (e.g., a sheet thickness of 40  $\mu\text{m}$ ) by using the cooling roll having a small wall thickness (e.g., a wall thickness of 10 mm), and (b) the thick foil strip (e.g., a sheet thickness of 40  $\mu\text{m}$ ) by using the cooling roll having a large wall thickness (e.g., a wall thickness of 30 mm). The measurement position for the temperature is defined in a position located on an upstream of the puddle, or a position located 20 cm distant from the puddle, for example. In this specification, either the cooling roll having a large wall thickness or simply a thick wall roll means the cooling roll having a wall thickness equal to or above 25 mm. Also, a conventional thin wall roll means the cooling roll having a wall thickness around 10 mm or less.

As shown in (a) and (b) in FIG. 8, in any of the case of using the thin wall roll and the case of using the thick wall roll, the temperature rises rapidly at an initial stage of casting. Then, the rate of temperature rise is stabilized but the temperature continues to rise linearly at a certain gradient.

In the case of the cooling roll having a small wall thickness, a microscopic structure of the foil strip to be formed remains amorphous up to a roll surface temperature  $T_{af1}$  but crystallization begins in excess thereof. As time advances further, a puddle break occurs at  $T_{pb1}$  and no foil strips will be formed thereafter. Although the same tendency applies in the case of the cooling roll having a large wall thickness, the time to the start of crystallization and the time to occurrence of the puddle break are considerably extended.

Moreover, both of the surface temperature  $T_{af}$  of the cooling roll at which crystallization begins and the roll surface temperature  $T_{pb}$  at which the puddle break occurs become higher in the case of the thick wall roll. That is,  $T_{af1} < T_{af2}$  and  $T_{pb1} < T_{pb2}$ . The reason is that the thick wall portion of the thick wall roll has a heat storage effect. Although a quench is required in the temperature zone from the melting point  $T_m$  to the glass transition temperature  $T_g$  in order to form the amorphous body, the conventional thin wall roll cannot deal with the quench when the foil strip becomes thicker. Even if a diameter of the roll is increased, it is not possible to absorb a heat flow in the above-mentioned temperature zone because the thin wall roll has a small heat capacity.

Moreover, the thick wall roll has large cooling power even when the temperature of the outer circumferential surface of the roll is high. The reason is that the heat flows more three-dimensionally in the thick wall roll (see arrows representing the heat flow in FIGS. 9A and 9B).

FIGS. 9A and 9B are views schematically showing temperature distribution in the direction of the wall thickness of the cooling roll immediately below the foil strip at one point in the temperature zone in which the temperature of the foil strip transits from  $T_m$  to  $T_g$  when casting the thick foil strip.

FIG. 9A shows the thin wall roll and FIG. 9B shows the thick wall roll. As shown in FIG. 9A, regarding the thin wall roll, the temperature of the outer circumferential surface of the roll is high and the temperature of the inner surface of the roll that contacts the cooling water is also high. On the other hand, as shown in FIG. 9B, both of a temperature  $T_{r2}$  of the outer circumferential surface and a temperature  $T_{w2}$  of the inner surface of the thick wall roll are lower than those  $T_{r1}$  and  $T_{w1}$  of the thin wall roll because the heat is widely diffused in a semi-three-dimensional manner in the case of the thick wall roll. As the inner surface temperature of the thick wall roll is lower than that of the thin wall roll, the amount of discharged heat between the roll and cooling water become  $Q_a > Q_b$ , and hence the cooling efficiency of the cooling water becomes lower in the case of the thick wall roll. However, the thick wall cooling zone has a larger heat capacity to be stored in the thick wall portion, whereby the time from the start of casting to the start of crystallization becomes longer.

As described above, the thick wall roll can store a large amount of heat temporarily by way of its own heat capacity. A large part of the heat stored in the thick wall portion of the cooling roll is transmitted and discharged to the cooling water while the roll goes around. However, part of the heat is accumulated in the cooling roll and raises the roll temperature. In order to accelerate the heat discharge from the cooling roll to the cooling water  $W$ , it is effective to increase the diameter and the width of the roll. Moreover, it is effective to maintain the cooling water at a low temperature. It is possible to extend the time available for continuous casting by taking these measures.

The diameter and the width of the cooling roll 113 can be designed based on the above-described heat transfer mechanism. Specifically, as the thick wall portion of the cooling roll 113 becomes thicker, the gradient of the straight line portion in the temperature curve of the outer circumferential surface of the cooling roll shown in FIG. 8 becomes larger. In order to reduce this gradient and to extend the time to a casting change, it is effective to increase the diameter and the width of the cooling roll 113. This is because time within one round to allow the inner surface of the cooling roll to contact the cooling water becomes longer by increasing the diameter of the cooling roll 113 and the amount of heat to be transmitted from the cooling roll to the cooling water is thereby increased.

In this embodiment, the diameter of the cooling roll 113 is set preferably in a range from 0.4 to 2.0 m. It is possible to ensure sufficient time within one round of the cooling roll by setting the diameter of the cooling roll 113 equal to or above 0.4 m. As a result, the heat transmitted from the molten alloy to the outer circumferential surface of the cooling roll 113 is efficiently discharged to the cooling water. In the meantime, by setting the diameter of the cooling roll 113 equal to or below 2.0 m, it is possible to facilitate an operation while avoiding an excessive increase in size of the production apparatus 101. Moreover, it is possible to facilitate ensuring strength of mechanical portions such as the bearings of the cooling roll 113.

It is preferable to set the width of the cooling roll 113 equal to 1.5 times or more of the width of the foil strip  $S$ , which is intended to be produced. In this way, the heat transmitted from the molten alloy  $A$  to the cooling roll 113 is also spread in the width direction and the amount of heat discharged to the cooling water for each round of the cooling roll is increased.

It is preferable to cool the cooling water  $W$  down in order to further enhance the cooling efficiency of the cooling roll. The temperature of the cooling water  $W$  to be supplied into the cooling roll 113 is set preferably equal to or below 20° C. or more preferably equal to or below 10° C. Because, as the

temperature of the cooling water is lower, it is possible to cool the cooling roll 113 down efficiently, thereby increasing the sheet thickness of the producible amorphous alloy foil strip. It is also possible to lower the freezing point by dissolving solute in the cooling water so as to set the temperature of the cooling water W equal to or below 0° C. upon supply into the cooling roll 113.

There may be a risk of causing dew condensation if the temperature of the outer circumferential surface of the cooling roll 113 becomes lower than a room temperature. In order to prevent dew condensation, gas that contains no moisture such as dry air or nitrogen may be sprayed onto the outer circumferential surface of the cooling roll. The spray of the gas should take place before the start of casting. Once the casting is started, the temperature of the outer circumferential surface of the cooling roller exceeds the room temperature soon, so it is no longer necessary to spray the gas.

Further, a material of the cooling roll 113 preferably has a large thermal conductivity. For example, the material has the thermal conductivity preferably equal to or above 250 W/mK, and more preferably equal to or above 300 W/mK. However, the material having the large thermal conductivity tends to have poor mechanical strength or abrasion resistance. Therefore, if the strength or hardness of the circumferential surface of the cooling roll is inadequate, it is also possible to harden only a surface layer of the circumferential portion. Hardening of the surface layer can be achieved by ion implantation, for example. In this case, it is preferable to provide implanted ions with a concentration gradient in order to prevent occurrence of a crack attributable to a heat stress.

The nozzle 115 used in production of the amorphous alloy foil strip according to this embodiment is a slit nozzle, and the width of a slit measured along the circumferential direction of the cooling roll 113 is in a range from 0.2 to 1.2 mm, e.g., in a range from 0.3 to 0.8 mm. Regarding the type of the slit, a single slit is acceptable but multiple slits are more preferable in light of productivity. From an empirical point of view, the sheet thickness is inversely proportional to the roll circumferential velocity. Therefore, in the case of the single-slit nozzle, it is necessary to set up the circumferential velocity slower than that of the multiple-slit nozzle. The circumferential velocity of the cooling roll 113 is set, for example, in a range from 10 to 30 m/sec., e.g., in a range from 15 to 25 m/sec. A distance (a gap) between the nozzle 115 and the outer circumferential surface of the cooling roll is set, for example, in a range from 0.1 to 0.5 mm, e.g., in a range from 0.15 to 0.25 mm. An ejection pressure of the molten alloy A is set, for example, in a range from 10 to 40 kPa, e.g., in a range from 20 to 30 kPa.

When starting the supply (pouring) of the molten alloy A onto the outer circumferential surface of the cooling roll 113 via the nozzle 115, the temperature of the outer circumferential surface of the cooling roll is gently increased except immediately after the start of pouring. Even if the temperature of the outer circumferential surface of the cooling roll 113 is increased, the sheet thickness of the foil strip remains almost constant as long as the temperature is equal to or below 200° C., for example, thereby ensuring the cooling rate necessary for forming the amorphous body. That is, the amorphous alloy foil strip S is obtained. Here, measurement of the temperature of the outer circumferential surface of the cooling roll is performed in a position in the center of the roll width and located 20 cm away on the upstream side from the puddle P. A contact-type thermometer is used for measuring the temperature of the outer circumferential surface of the cooling roll, for example. A concrete example is disclosed in Patent Document 3.

The timing to change casting may also be determined by measuring a surface temperature of the formed foil strip S. A position of measurement is preferably located in an appropriate position prior to detachment of foil strip S from the cooling roll. Although the above-described contact-type thermometer is applicable to this measurement, it is also possible to use an infrared radiation thermometer in the case of the iron-base alloy. Monitoring the temperature of the foil strip S is a more straightforward measure for judging the amorphous property of the foil strip in the course of casting.

Here, in the production apparatus 101 according to this embodiment, it is also possible to use only one side of the cooling rolls 113 to perform casting intermittently. Specifically, casting of the foil strip is performed in a state of rotating the cooling roll and supplying the cooling water and then the supply of the molten alloy is stopped if the temperature of the outer circumferential surface of the cooling roll reaches a predetermined value. At this time, rotation of the cooling roll and the supply of the cooling water are continued. By stopping the casting and continuing the supply of the cooling water, the temperature of the outer circumferential surface of the cooling roll is rapidly cooled down. Thereafter, the casting is resumed at a time point when the temperature of the outer circumferential surface of the roll is back to the room temperature, for example. In this way, it is possible to produce the thick amorphous alloy foil strips in an industrial scale by use of the single cooling roll, although intermittently.

Next, effects of this embodiment will be described.

In this embodiment, the production apparatus 101 for an amorphous alloy foil strip is provided with the two cooling rolls 113a and 113b and the foil strips S are cast by alternately using these rolls. In this way, the single cooling roll repeats casting and cooling down, whereby it is possible to set the temperature equal to or below the predetermined value. As a result, it is possible to cast the amorphous alloy foil strip having a large sheet thickness almost continuously and to perform production in an industrial scale. Such an amorphous alloy foil strip is applicable to a power transformer or a core of a motor, for example, and is also applicable to a magnetic shield material.

Moreover, since the multiple-slit nozzle is used as the nozzle 115 in this embodiment, it is possible to equalize the sheet thickness of the foil strips S and to reduce occurrence of pin holes. A surface condition of the foil strip S is microscopically rough due to minute vibration of the puddle P, a local defect of the cooling roll 113, and the like. Significant roughness leads to formation of scale-like stripes called fish scales or of pin holes on the foil strips S, which are macroscopically observable. By using the multiple-slit nozzle method, these defects formed on a fluid layer drawn out of the puddle on the upstream side are compensated by the puddle on the downstream side. Therefore, it is possible to produce the foil strips S having favorable surface conditions with very few pin holes.

As described above, the surface of the amorphous alloy foil strip produced in accordance with the multiple-slit nozzle method is smooth with very few pin holes. A number density of pin holes on the foil strip is equal to or below 25 holes/m<sup>2</sup>, for example, or equal to or below 10 holes/m<sup>2</sup>, for example, or none, for example. A space factor is improved when stacking the foil strips due to the decrease of pin holes, the smoothed surface, and so forth. For example, according to this embodiment, the space factor becomes equal to or above 80% when the foil strip having a sheet thickness equal to or above 33 µm is produced and then a wound iron core is fabricated by using this foil strip; the space factor becomes equal to or above 85% when the foil strip having a sheet thickness equal to or above

## 15

40  $\mu\text{m}$  is produced and then a wound iron core is fabricated by using this foil strip; and the space factor becomes equal to or above 90% when the sheet thickness is equal to or above 45  $\mu\text{m}$ . Moreover, the space factor becomes equal to or above 93% in the case of the foil strip having a sheet thickness equal to or above 50  $\mu\text{m}$ . The foil strip having the smooth surface and very few pin holes causes a smaller hysteresis loss as there are fewer obstacles for domain wall motion, and is therefore a favorable material for an electromagnetic iron core. In addition, an improvement in the space factor has the same significance as an improvement in a saturation magnetic flux density  $B_s$ . For example, an improvement in the space factor from 80% to 90% has practically the same effect as an improvement in  $B_s$  from 1.60 T to 1.78 T.

In this embodiment, the production apparatus 101 applies the cooling rolls 113 having a large wall thickness and mechanical strength of the cooling rolls is high. Accordingly, it is possible to minimize occurrence of variations in the sheet thickness and characteristics of the foil strip S attributable to uneven thermal expansion of the cooling rolls and to produce the homogeneous amorphous alloy foil strips. Also, by using the cooling rolls having a large wall thickness, it is possible to eliminate various problems that occur frequently in the case of the conventional thin wall rolls, which are attributable to uneven thermal deformation of the rolls. For example, local embrittlement or fluctuation in magnetic characteristics of the foil strips S due to uneven cooling of the foil strips or the like does not occur.

Next, a second embodiment of the invention will be described.

FIG. 10 is a perspective view showing a structure of cooling rolls 113. As shown in FIG. 10, in a production apparatus 102 for an amorphous alloy foil body, the cooling roll 113 is hollow and an opening 120 is formed at a central part of a side surface 119 on an opposite side (hereinafter referred to as a "water supply side") of a side where the driving unit 111 is disposed (hereinafter referred to as a "driving side"). The shape of the opening 120 is circular and a central axis thereof conforms to a central axis of the cooling roll 113. That is, the cooling roll 113 has a shape of an open roll.

A cross section of the cooling roll from the outer circumferential surface toward the central axis is shown in FIG. 11. On an inner circumferential surface 121 of the cooling roll in FIG. 11, multiple partition plates 122 extending along the circumferential direction of the cooling roll 113 and spaces defined by the side surface 119 on the water supply side, the multiple partition plates 122, and a side surface 123 on the driving side are respectively formed into water channels 124.

A water supply pipe 125 and a drain pipe 126 are brought into the cooling roll 113 via the opening 120. The water supply pipe 125 is connected to a water supply unit (not shown) and the drain pipe 126 is connected to a pump (not shown). Branch pipes 125a in the same number as the water channels 124 are branched off from the water supply pipe 125 and the cooling water is supplied to the respective water channels 124 via the respective branch pipes. Likewise, branch pipes 126a in the same number as the water channels 124 are branched off from the drain pipe 126 and the cooling water is discharged from the respective water channels 124 via the respective branch pipes 126a. A shape of a cross section orthogonal to a longitudinal direction in the branch pipe 126a has a streamlined shape along the circumferential direction of the cooling roll 113, for example. In this way, the cooling roll 113 functions as a water-cooled roll configured to circulate the cooling water W inside.

Next, operations of the second embodiment will be described.

## 16

First, as shown in FIG. 10, the cooling rolls 113a and 113b are rotated by way of the rotating shaft members 112a and 112b by driving the driving unit 111. At this time, the rotating speed of the cooling rolls 113 is set to a rotating speed so as to render a centrifugal force in the water channels 124 greater than the gravity.

In this state, as shown in FIG. 11, the cooling water W is supplied to the respective water channels of the cooling rolls 113a and 113b via the water supply pipes 125. In this way, the 10 cooling water W inside the respective water channels 124 is rotated together with the cooling rolls 113 and reaches all parts of the water channels 124. That is, the cooling water W sticks to the inner surfaces of the cooling rolls 113 by the centrifugal force and does not fall off even at upper parts of 15 the cooling rolls 113. At this time, tip ends of the branch pipes 126a are inserted to the cooling water W.

On the other hand, the cooling water is discharged from the respective water channels 124 via the drain pipe 126 by operating the pump (not shown). In this way, a constant amount of 20 the cooling water W is retained inside the cooling rolls 113. At this time, since the water channels 124 are open toward the center of the cooling rolls 113, surfaces of the cooling water W on the central side of the cooling rolls 113 constitute free surfaces.

25 Then, as shown in FIG. 10, the crucible 114 is located beside one of the cooling rolls 113, e.g., the cooling roll 113a, by use of the moving unit 116. Then, the molten alloy A is ejected from the nozzle 115 toward the outer circumferential surface of the cooling roll through the slit 117 so as to come in contact 30 with the outer circumferential surface of the cooling roll 113a. In this way, the puddle P is formed between the slit 117 and the cooling roll 113a. Then, a portion of the molten alloy A forming the puddle P, which contacts the cooling roll 113a, is cooled down so as to increase viscosity and is drawn by the 35 circumferential surface of the cooling roll 113a and cooled down by the cooling roll 113a while moving in the rotating direction of the cooling roll 113a, and is formed into a super-cooled metallic fluid and then solidified and cooled down below the glass transition point to form the amorphous alloy 40 foil strip S. The cooling rate at this time is equal to or above  $1 \times 10^5^\circ\text{C./sec.}$ , for example.

The heat transmitted from the molten alloy A to the cooling roll 113a is transferred from the cooling roll 113a to the cooling water W through the inside of the roll. Then, the heat 45 transmitted to the cooling water W is discharged to the outside of the cooling roll together with the cooling water W through the drain pipe 126. That is, the heat of the molten alloy A is discharged by way of the molten alloy A  $\rightarrow$  the cooling roll 113a  $\rightarrow$  the cooling water W.

50 The temperature of the cooling roll 113a is gradually increased along with casting of the foil strips S. When the temperature of the outer circumferential surface of the cooling roll reaches a predetermined value, the nozzle 115 is closed to stop ejection of the molten alloy A. Next, the crucible 114 is moved along the rail of the moving unit 116 and is located beside the other cooling roll 113, i.e., the cooling roll 113b. Then, the nozzle 115 is opened to eject the molten alloy A toward the outer circumferential surface of the cooling roll 113b. In this way, the foil strip S is cast with the 55 cooling roll 113b by the same operation as the above-described operation with the cooling roll 113a. Specifically, as shown in FIG. 4, the cooling roll used for casting the foil strips S is switched from the cooling roll 113a to the cooling roll 113b. Although the cooling roll 113a is in the standby state in 60 this period, the cooling water W is continuously supplied to the cooling roll 113a as well to cool the cooling roll 113a down.

Thereafter, when the temperature of the cooling roll 113b reaches the predetermined value, the cooling roll used for casting the foil strips S is switched from the cooling roll 113b to the cooling roll 113a. By this time, the cooling roll is sufficiently cooled down so that it is possible to resume casting the foil strip S. Here, the cooling water W is continuously supplied to the cooling roll 113b in the standby state as well in this period to continue cooling. Likewise, as shown in FIG. 4, the cooling roll 113a and the cooling roll 113b are alternately used thereafter to continue production of the foil strips S.

A mechanism for cooling the cooling rolls used in the second embodiment is heat transmission by convection of the cooling water. As the cooling rolls 113 are rotated at the high speed, the strong centrifugal force is applied to the cooling water. The magnitude of this centrifugal force is 50 to 150 times as large as the gravity. For this reason, the temperature rises at a portion of the cooling water located close to the roll and large buoyancy acts on this portion where the density is reduced. This action forms a driving force to generate forcible convection. Accordingly, the cooling water has a sufficient heat transmitting effect although it remains almost stationary relative to the rolls.

Moreover, since the open roll is used as the cooling roll in this embodiment, no air bubbles remain on the inner surface of the cooling roll. The air bubbles come up and disappear on the free surface by the strong centrifugal force. In a method of feeding water through an embedded water channel, there may be a case in which quality of material of a formed foil strip is partially deteriorated by an influence of uneven cooling attributable to residual air. Configurations, operations, and effects of this embodiment other than those mentioned above are similar to the above-described first embodiment.

Next, a variation 1 of the second embodiment will be described. A cooling roll used in this variation 1 applies an open roll structure which is hollow inside and open on one of side surfaces. Moreover, the multiple water channels 124 extending in the circumferential direction of the cooling roll are formed by providing an inner circumferential surface with the partition plates 122. Further, as shown in FIG. 12A, each of the water channels 124 including a valve 144 is provided with the branch pipe 125a of the water supply pipe 125 and the branch pipe 126a of the drain pipe 126. In this way, it is possible to adjust a flow rate of the cooling water depending on the water channel 124, i.e., depending on the position in the width direction of the cooling roll 113, and to control a heat flow rate. Moreover, it is possible to set up a different water temperature depending on the water channel. By using this configuration, it is possible to equalize temperature distribution in the width direction of the cooling roll 113 and to equalize the cooling power in the width direction of the cooling roll.

FIG. 12B shows a cross-section of another cooling roll 130 used in the variation 1. As shown in FIG. 12B, in the cooling roll 130, each water channel is provided with three fins 128, for example. Each of partition plates 127 and the fins 128 extends in the circumferential direction and a cross section orthogonal to the longitudinal direction is in a triangular shape. The heights of the fins are set lower than the heights of the partition plates so as to be submerged. It is possible to further enhance heat transfer efficiency by providing the fins 128.

Next, a variation 2 of the second embodiment will be described.

FIG. 13 is a cross-sectional view illustrating the vicinity of a cooling roll of a production apparatus 103 for an amorphous alloy foil strip according to this variation. As shown in FIG.

13, in the production apparatus 103 for an amorphous alloy foil strip according to this variation, a pair of cooling rolls 133 are provided on both sides of the driving unit 111 (see FIG. 10) as similar to the production apparatus 102 according to the above-described second embodiment.

Moreover, the drain pipe 126 (see FIG. 10) is not brought into the cooling roll 133 but through holes 134 to feed the cooling water from the water supply side toward the outer circumferential direction are formed at portions distant from the driving side of the cooling roll 133. Also, a convex portion 135 having a cross section of a convex shape is provided along the outer circumferential surface of the cooling roll at a portion closer to the driving side than the through holes 134. In addition, a flange 136 is provided so as to cover an end on the water supply side of the cooling roll 133, i.e., the portions where the through holes 134 and the convex portion 135 are provided. The flange 136 is not in contact with the cooling roll 133 but is fixed to a floor surface. A drain outlet 137 is provided at a bottom of the flange 136.

Furthermore, an entrance port is provided on a side surface of the flange 136 and a water supply pipe 139 is brought into the cooling roll 133 through this entrance portion 138 and the opening 120. The water supply pipe 139 is not provided with any branch pipes and is configured to supply the cooling water W to a portion on the driving side in the cooling roll 133. Moreover, no partition walls 122 (see FIG. 11) are formed in the inner circumferential surface of the cooling roll 133. Configurations of this variation other than those mentioned above are similar to the production apparatus 102 (see FIG. 10) according to the above-described second embodiment.

Next, operations of the production apparatus 103 according to this variation will be described.

In this variation, the cooling water W supplied into the cooling roll 133 via the water supply pipe 125 sticks to the inner circumferential surface of the cooling roll 133 by the centrifugal force and moves from the driving side to the water supply side along an axial direction of the cooling roll 133 while being rotated in the circumferential direction of the cooling roll 133 together with rotation of the cooling roll 133. In this process, heat exchange with the cooling roll 133 takes place. Then, the cooling water W is discharged out of the cooling roll 133 via the through holes 134 by the centrifugal force. The cooling water W discharged from the through holes 134 is received by the flange 136 and collected at a lower part of the flange 136 by way of the gravity, and is discharged via the drain outlet 137. Operations of this variation other than those mentioned above are similar to the above-described second embodiment. That is, the foil strips S are cast by alternately using the pair of cooling rolls 133.

Next, effects of this variation will be described.

In this variation, it is not necessary to insert the drain pipe into the cooling water W which is rotated at the high speed inside the cooling rollers 133. Therefore, vibration and the like attributable to resistance of the water hardly occurs and mechanical reliability is high. Moreover, the water flow of the cooling water W is stabilized. Effects of this variation other than those mentioned above are similar to the above-described second embodiment.

Here, it is also possible to provide fins inside the cooling roll 133 in order to increase a contact area with the cooling water W. In this case, notches are formed on the fins in order to render the cooling water W movable along the axial direction of the cooling roll 133. In this way, it is easy to discharge the cooling water W which is warmed up.

Next, a third embodiment of the invention will be described.

FIG. 14 is a front view illustrating a production apparatus for an amorphous alloy foil strip according to this embodiment. FIG. 15 is a cross-sectional view illustrating the structures of a cooling roll and cooling zones in FIG. 14. FIG. 16 is a conceptual diagram showing a pathway of cooling water circulated in the cooling roll in FIG. 14. FIG. 17 is a timing chart illustrating a method for producing an amorphous alloy foil strip according to this embodiment in which a horizontal axis indicates time and a vertical axis indicates the cooling zones.

As shown in FIG. 14, a production apparatus 201 for an amorphous alloy foil strip according to this embodiment is configured to mainly produce the iron-base amorphous alloy foil strip S as similar to the first embodiment. Compositions of the foil body S to be produced in this embodiment are similar to the above-described first embodiment, which are the compositions shown in FIG. 5, for example.

A cooling roll 213 having a large wall thickness configured to circulate cooling water inside is disposed in the production apparatus 201. The cooling roll 213 is rotatably supported by rotating shaft members 212a and 212b (hereinafter also collectively referred to as “rotating shaft members 212”), and the rotating shaft members 212 are connected to a driving unit 211 which shares a common rotating axis. A motor (not shown) is embedded in the driving unit 211 and is configured to rotate the cooling roll via the rotating shaft members 212. The rotating shaft members 212 and the cooling roll 213 are supported by bearings 241a and 241b.

As shown in FIG. 14 and FIG. 15, two cooling zones 213a and 213b, which have a heat insulating zone 218 interposed therebetween, are provided in an outer circumferential portion of the cooling roll 213. The cooling zones 213a and 213b are fixed to a supporting mechanism 231 made of a metallic alloy having large strength. The shape of the cooling zones 213a and 213b is a ring shape surrounding the outer circumferential portion of the cooling roll 213 and having a predetermined thickness, which are separated from each other in an axial direction of the cooling roll 213. Also, the heat insulating zone 218 is disposed between the cooling zone 213a and the cooling zone 213b, and the thickness thereof is set equal to or above 50% of the respective thicknesses of the cooling zones 213a and 213b. For example, the outer circumferential surfaces of the cool zone 213a and 213b and of the heat insulating zone 218 form a continuous surface. The supporting mechanism 231 is coupled with the roll driving unit 211, whereby the cooling roll 213 is provided with a torque by the roll driving unit 211.

The cooling zones 213a and 213b are made of metal or an alloy having high thermal conductivity, and are made of copper or a copper alloy, for example. The thermal conductivity of copper is equal to 395 W/(m·K) at 100° C. Alternatively, the cooling zones 213a and 213b may be made of either a Be—Cu alloy or a Cr—Cu alloy, and the thermal conductivity of these copper alloys ranges from 150 to 300 W/(m·K).

On the other hand, the heat insulating zone 218 is made of a material having lower thermal conductivity than the material for forming the cooling zones 213a and 213b, and is made of a material having the thermal conductivity equal to or below 3 W/(m·K), for example. The heat insulating zone 218 is made of, for example, a refractory brick (thermal conductivity: 1.1 W/(m·K)), a porcelain (thermal conductivity: 1.5 W/(m·K)), glass (thermal conductivity: 1.4 W/(m·K)), or asbestos (thermal conductivity: 0.3 W/(m·K)).

The production apparatus 201 is provided with a crucible 214 for retaining the molten alloy A (see FIG. 3), and a nozzle 215 for ejecting the molten alloy A in the crucible 214 to the outside of the crucible 214 is fitted to a lower end of the

crucible 214. Here, an ejection portion of the nozzle 215 is disposed closely to the outer circumferential surface of the cooling roll 213. Configurations of the crucible 214 and the nozzle 215 are similar to the configurations of the crucible 114 and the nozzle 215 (see FIG. 2) in the above-described first embodiment. The nozzle 215 is a multiple-slit nozzle, for example.

Further, the production apparatus 201 is provided with a moving unit 216 for moving the crucible 214 along the axial direction of the cooling roll 213. The moving unit 216 moves the crucible 214 between a position where the nozzle 215 faces the cooling zone 213a and a position where the nozzle 215 faces the cooling zone 213b.

FIG. 16 shows a simplified pathway of cooling water W in the production apparatus for an amorphous alloy foil strip according to this embodiment. In the production apparatus 201, in order to retain the cooling water lower than a predetermined temperature such as a room temperature during casting, cooling units 243 configured to cool the cooling water down are provided in the course of the pathway of the cooling water W, e.g., in a water tank 242. The cooling water is supplied from the water tank 242 to water channels 224 of the cooling roll 213 by use of water supply pipes 225, and after circulation in the cooling roll 213, is returned from the water channels 224 to the water tank 242 via drain pipes 226. Then, the cooling water is cooled down by the cooling units 243 in the course of the circulation. Here, no water channel 224 is formed inside the heat insulating zone 218.

Configurations of the water supply pipes 225 and the drain pipes 226 are not limited to the configurations shown in FIG. 15. It is possible to apply any configurations connectable to the cooling roll 213. For example, as shown in FIG. 15, the water supply pipe 225 and the drain pipe 226 may constitute a double pipe. In this case, the cooling zone 213a and the cooling zone 213b are respectively provided with a cooling water circulation system, which includes the water tank 242, the cooling unit 243, the water supply pipe 225, the water channel 224, and the drain pipe 226, independently of each other. This is intended for thermally separating the cooling zone 213a from the cooling zone 213b. Alternatively, it is also possible to connect the water supply pipe 225 to one end of the cooling roll 213 in the axial direction and to connect the drain pipe 226 to the other end. In this case, the water supply pipe 225 pierces a central part 232 of the supporting mechanism 231 of the cooling roll 213 in the axial direction. Moreover, as viewed from the axial direction of the cooling roll 213, the water channels on a water supply side are branched off from the center toward the outer circumferential surface of the cooling roll 213 in two mutually opposite directions and the water channels on a drain side are merged from two directions which are orthogonal to a direction of extension of the branches on the water supply side from the outer circumferential surface toward the center of the cooling roll 213. That is, as viewed from the axial direction of the cooling roll 213, the branches connecting the central part to an outer circumferential portion of the cooling roll 213 is formed into a cruciform.

Next, operations of the production apparatus 201 according to this embodiment configured as described above, that is, a method for producing an amorphous alloy foil strip according to this embodiment will be described.

First, as shown in FIG. 14, the cooling roll 213 is rotated by way of the rotating shaft members 212 by driving the driving unit 211. Next, the nozzle 215 is located closely to the outer circumferential surface of one of the cooling zones on the cooling roll 213, e.g., the cooling zone 213a, while providing a given interval. Then, the molten alloy A is ejected from the

crucible 214 via the nozzle 215. In this way, a puddle P is formed between the nozzle 215 and the cooling zone 213a. Then, of the molten alloy forming the puddle P, the molten alloy located in the vicinity of a contact surface with the cooling zone 213a is cooled down so as to increase viscosity and is drawn out of the puddle P by rotation of the cooling roll 213. The alloy thus drawn out is a supercooled liquid at this point, but is quenched by the cooling roll 213 down to a glass transition temperature or below and is formed into the amorphous alloy foil strip S. A cooling rate required for rendering the foil strip (or the supercooled liquid) drawn out of the puddle P amorphous is equal to or above  $1 \times 10^5$  °C./sec. in the case of the iron-base alloy, for example.

The heat transmitted from the molten alloy and the foil strip to the cooling zone 213a in order to form the amorphous alloy foil strip is transferred from the outer circumferential portion of the cooling zone 213a into the cooling roll 213 and transmitted to the cooling water circulated inside the water channel 224. Then, the heat transmitted to the cooling water is collected by the water tank 242 together with the cooling water via the drain pipe 226. That is, the heat of the molten alloy A is discharged by way of the molten alloy A → the cooling roll 213 → the cooling water W.

Thereafter, when the temperature of the cooling zone 213a reaches a predetermined value (Th) along with casting of the foil strip S, the nozzle 215 is closed to stop ejection of the molten alloy A. After the stop, the moving unit 216 promptly moves the crucible 214 close to the outer circumferential surface of the cooling zone 213b. Then, the supply of the molten alloy A is resumed. In this way, a foil strip S is cast by using the cooling zone 213b. At this time, the cooling zone 213b is gradually heated along with casting of the foil strips S, the cooling zone 213a is rapidly cooled down by the cooling water. Thereafter, when the temperature of the cooling zone 213b reaches the predetermined value (Th), the supply of the molten alloy A is stopped and the crucible 214 is promptly moved close to the outer circumferential surface of the cooling zone 213a again. Then, the molten alloy is supplied. By this time, the cooling zone 213a is sufficiently cooled down and reaches the room temperature, for example. When the temperature of the cooling zone 213a exceeds the predetermined value (Th) again, the supply of the molten alloy A is stopped and the crucible 214 is promptly moved to the position corresponding to the cooling zone 213b to continue casting. By alternating the above-described actions, it is possible to ensure the cooling rate necessary for forming the amorphous body. This is particularly effective for production of foil strips having a large sheet thickness (equal to or above 30 µm). In contrast, it has not been possible to perform continuous casting for a long period of time to form thick foil strips equal to or above 30 µm because the cooling roll having a single cooling zone has been used previously.

Although the above-described example has exemplified the aspect of moving the crucible 214 from the position facing the cooling zone 213a to the position facing the cooling zone 213b, it is also possible to move the cooling zone to face the nozzle 215 from the cooling zone 213a to the cooling zone 213b by moving the cooling roll 213 along the rotating axis thereof.

Accordingly, by repeating a first process of supplying the molten alloy A to the outer circumferential surface of the cooling zone 213a while rotating the cooling roll 213 and a second process of stopping the supply of the molten alloy A, moving the crucible 214 to the position facing the outer circumferential surface of the cooling zone 213b, and supplying the molten metal A to the outer circumferential surface of the cooling zone 213b, it is possible to produce the amorphous

alloy foil strip having a large sheet thickness almost continuously in an industrial scale. An operation style in this embodiment is illustrated in FIG. 17. As shown in FIG. 17, when casting is performed by using one of the cooling zones, the other cooling zone is in a cooling process by using the cooling water.

Next, the production apparatus and the production method according to this embodiment will be described in detail.

Heat capacities of the cooling zones 213a and 213b of the cooling roll 213 are designed based on the heat transfer mechanism explained in conjunction with the above-described first embodiment. It is effective to increase the heat capacities of the cooling zones 213a and 213b in order to extend the time to the start of crystallization and the time to the interruption of pouring in FIG. 8. This means nothing but increasing the wall thickness, the diameter, and the width of the cooling zones.

Each of the cooling zones 213a and 213b preferably has a wall thickness equal to or above 25 mm. The reason for this is similar to the reason for setting the wall thickness 129 (see FIGS. 6A to 6C) of the cooling roll 113 equal to or above 25 mm in the above-described first embodiment. Also, the diameter of the cooling zones 213a and 213b is set preferably in a range from 0.4 to 2.0 m. It is possible to ensure sufficient time within one round of the cooling zone by setting the diameter of the cooling zones 213a and 213b equal to or above 0.4 m. As a result, the heat transmitted from the molten alloy to the outer circumferential surface of the cooling zone is efficiently discharged to the cooling water. On the other hand, by setting the diameter of the cooling zones equal to or below 2.0 m, it is possible to facilitate an operation while avoiding an excessive increase in size of the production apparatus 201. Moreover, it is possible to facilitate ensuring strength of mechanical portions such as the bearings of the cooling roll 213.

Also, it is preferable to set the width of each of the cooling zones 213a and 213b equal to 1.5 times or more of the width of the foil strip S, which is intended to be produced. In this way, the heat transmitted from the molten alloy A to the cooling zones 213a and 213b is also spread in the width direction and the amount of heat discharged to the cooling water for each round of the cooling roll is increased.

Further, the material of the cooling zones 213a and 213b preferably has a large thermal conductivity. For example, the material has the thermal conductivity preferably equal to or above 250 W/(m·K) and more preferably equal to or above 300 W/(m·K). The uneven thermal deformation of the roll, which has been the problem of the conventional thin wall roll, hardly occurs by increasing the wall thickness of the cooling zones 213a and 213b. Accordingly, it is possible to select the material while placing more emphasis on the thermal conductivity than the mechanical strength. However, the material having the large thermal conductivity tends to have poor abrasion resistance. It is possible to achieve both the abrasion resistance and the high thermal conductivity by carrying out the process to harden only the surface layer of the circumferential portion of the cooling roll in order to retain the abrasion resistance. Hardening of the surface layer can be achieved by ion implantation, for example. In this case, it is preferable to provide implanted ions with a concentration gradient in order to prevent occurrence of a crack attributable to a heat stress.

On the other hand, the reason for providing the heat insulating zone 218 is to reduce the amount of heat flowing to the adjacent cooling zone. A temperature gradient in the width direction of the cooling zone occurs if this amount of heat is significant, and this may cause deviation of the sheet thickness in the width direction of the foil strip. Therefore, it is preferable to increase the wall thickness (a depth) of the heat

insulating zone 218 as much as possible. The wall thickness of the heat insulating zone 218 is preferably equal to or above 50% of the wall thickness of the cooling zones, and is more preferably equal to the wall thickness of the cooling zones. While the width of the heat insulating zone 218 depends on the thermal conductivity of the heat insulating zone, it is adequate to provide about 1 mm in the case of a refractory or a ceramic. In view of productivity, the width should be designed so as to render a time loss attributable to the nozzle movement as little as possible.

The material of the heat insulating zone 218 is not particularly limited as long as the material has heat resistance and low thermal conductivity. Refractory and ceramics such as BN or  $\text{Al}_2\text{O}_3$  are cited as examples. It is also possible to use only the air as the heat insulating zone 218 without using any specific material. In other words, it is possible to form the heat insulating zone 218 by using an air layer. The thermal conductivity of the air is equal to 0.03 W/(m·K). Accordingly, it is possible to achieve extremely high heat insulation. However, the molten alloy may be spilled on a groove between the cooling zones when moving the nozzle from one of the cooling zones to the other cooling zone. It is therefore preferable to cover the groove with a material having poor wettability to the molten alloy in order to avoid such a problem and not to cause a coagulation to adhere to the groove.

Here, it is also preferable to provide fins 228 in the inner surfaces of the water channels 224 as shown in FIG. 10 in order to further enhance the cooling effect of the cooling water W. By increasing the contact area between the cooling zone and the cooling water, it is possible to increase the amount of heat discharged of the cooling water W and to extend the time to the change of casting.

When starting the supply (pouring) of the molten alloy A onto the outer circumferential surface of one of the cooling zones, e.g., the cooling zone 213a, via the nozzle 215, the temperature of the outer circumferential surface of the cooling zone 213a is rapidly increased immediately after the start of pouring. Then, the rate of rise is reduced and the temperature is gently increased at a constant rate thereafter. Even if the temperature of the outer circumferential surface of the cooling zone 213a is increased, the sheet thickness of the foil strip remains almost constant as long as the temperature is equal to or below 200°C., for example, thereby ensuring the cooling rate necessary for forming the amorphous body. That is, the amorphous alloy foil strip is obtained. Here, the measurement of the temperature of the outer circumferential surface of the cooling zone is performed in a position in the center of the width of the cooling zone and located 20 cm away on the upstream side from the puddle P, for example. A contact-type thermometer is used for measuring the temperature of the outer circumferential surface of the cooling roll, for example. The concrete example is disclosed in Patent Document 3.

The timing to change casting between the cooling zones may also be determined by measuring the surface temperature of the formed foil strip S. A position of measurement is preferably located in an appropriate position prior to detachment of foil strip S from the cooling roll. Although the contact-type thermometer can be used as the thermometer for measuring the surface temperature of the foil strip S, it is also possible to use the infrared radiation thermometer in the case of the iron-base alloy. Monitoring the temperature of the foil strip S is a more straightforward measure for judging the amorphous property of the foil strip in the course of casting. It is also possible to employ a method of monitoring the temperature in a predetermined position on the outer circumferential surface of the cooling zone. In the case of the same

apparatus, it is also possible to set up time for the casting change based on the casting time with which the fine foil strip can be obtained. If the size (the sheet thickness and the width), the alloy composition, and the like of the amorphous alloy foil strip to be produced remain the same, it is also possible to perform the change based on time which is measured in advance.

Next, effects of this embodiment will be described.

In this embodiment, the cooling roll 213 of the production

10 apparatus 201 for an amorphous alloy foil strip is provided with the two cooling zones 213a and 213b and the foil strips S are cast by alternately using these zones. In this way, the single cooling zone repeats casting and cooling down, whereby it is possible to set the roll temperature equal to or 15 below the predetermined value. As a result, it is possible to produce the amorphous alloy foil strip having a large sheet thickness in an industrial scale. The amorphous alloy foil strip is applicable to a power transformer or a core of a motor, for example, and is also applicable to a magnetic shield material.

20 Moreover, in this embodiment, the cooling zone 213a and the cooling zone 213b are disposed distant from each other. Therefore, the cooling zones are thermally independent so that one of the cooling zones can be cooled down while the foil strips are cast in the other cooling zone. In addition, by 25 providing the heat insulating zone 218 between the cooling zone 213a and the cooling zone 213b, it is possible to enhance rigidity of the entire cooling roll 213 while maintaining the heat insulation between the cooling zone 213a and the cooling zone 213b.

30 Furthermore, according to this embodiment, it is possible to perform casting alternately by using the single cooling roll. Therefore, as compared to the above-described first and second embodiments, there is an advantage that it is only necessary to provide one set of the driving unit and the like. In this 35 way, equipment costs can be suppressed. On the other hand, since the two cooling rolls are provided according to the first and second embodiments, it is possible to thermally separate the cooling rolls more reliably and to rotate the cooling rolls at mutually different rotating speeds. Accordingly, there is an 40 advantage of increase in the degree of freedom of production.

45 Configurations, operations, and effects of this embodiment other than those mentioned above are similar to the above-described first embodiment. For example, since the multiple-silt nozzle is also used as the nozzle 215 in this embodiment, it is possible to equalize the sheet thickness of the foil strips S and to reduce occurrence of pin holes. For example, it is possible to control the number density of pin holes on the foil strip S equal to or below 25 holes/m<sup>2</sup>, for example, or equal to or below 10 holes/m<sup>2</sup>, for example, or none, for example. 50 Moreover, since this embodiment also applies the cooling zones having a large wall thickness, it is possible to resolve various problems attributable to the uneven thermal deformation of the cooling roll, which may occur frequently in the case of using the thin wall roll. For example, local embrittlement or fluctuation in magnetic characteristics of the foil strips S due to uneven cooling of the foil strips or the like does 55 not occur.

55 Next, a fourth embodiment of the invention will be described.

60 FIG. 19 is a front view illustrating a production apparatus for an amorphous alloy foil strip according to this embodiment. FIG. 20 is a cross-sectional view illustrating the structures of a cooling roll and cooling zones in FIG. 19. FIG. 21 is a conceptual diagram showing a pathway of cooling water circulated in the cooling roll in FIG. 19.

65 As shown in FIG. 19, a production apparatus 301 for an amorphous alloy foil strip according to this embodiment is

configured to mainly produce an iron-base amorphous alloy foil strip S. The compositions, the sheet thickness, and the width of the foil strip S are similar to the above-described first to third embodiments.

As shown in FIG. 19 and FIG. 20, a cooling roll 313 having a large wall thickness configured to circulate cooling water inside is disposed in the production apparatus 301. Two cooling zones 313a and 313b, which have a forbidden zone 318 interposed therebetween, are provided at an outer circumferential portion of the cooling roll 313. The cooling zones 313a and 313b are fixed to a supporting mechanism 331 made of a metallic alloy having large strength. The forbidden zone 318 is a portion in the outer circumferential surface of the cooling roll 313 where no molten alloy is supplied.

The cooling zones 313a and 313b are made of metal or an alloy having high thermal conductivity, and are made of, for example, copper or a copper alloy. The thermal conductivity of copper is equal to 395 W/(m·K) at 100° C. Alternatively, the cooling zones 313a and 313b may be made of either the Be—Cu alloy or the Cr—Cu alloy, and the thermal conductivity of these copper alloys ranges from 150 to 300 W/(m·K).

On the other hand, the forbidden zone 318 may be formed integrally with the cooling zones 313a and 313b by use of the same material or may be made of a different material from the cooling zones 313a and 313b. For example, when the forbidden zone 318 is made of a different material from the cooling zones 313a and 313b, thermal conductivity of such a material is set, for example, equal to or above 10 W/(m·K). For example, carbon steel (thermal conductivity: 48.5 W/(m·K)), 18-8 stainless steel (thermal conductivity: 16.5 W/(m·K)), and a copper alloy such as brass (thermal conductivity: 128 W/(m·K)) may be cited as the material for forming the forbidden zone 318.

FIG. 21 shows a simplified pathway of cooling water W in the production apparatus for an amorphous alloy foil strip according to this embodiment. Water channels 324 are formed inside the cooling roll 313. The water channels 324 are also formed inside the forbidden zone 318 in addition to the inside of the cooling zones 313a and 313b.

Configurations of this embodiment other than those mentioned above are similar to the above-described third embodiment. Specifically, the production apparatus 301 is provided with a moving unit 316 for moving a crucible 314 along the axial direction of the cooling roll 313. The moving unit 316 moves the crucible 314 between a position where a nozzle 315 faces the cooling zone 313a and a position where the nozzle 315 faces the cooling zone 313b. Moreover configurations of the water channels 324, water supply pipes 325 and drain pipes 326 may also apply various configurations as similar to the above-described third embodiment. In addition, the nozzle 315 is a multiple-slit nozzle, for example.

Next, operations of the production apparatus 301 according to this embodiment configured as described above, that is, a method for producing an amorphous alloy foil strip according to this embodiment will be described.

In this embodiment as well, the molten alloy A is supplied to the cooling zone 313a and the cooling zone 313b alternately by moving the crucible 314 by use of the moving unit 316, as in the case of the above-mentioned third embodiment. At this time, the molten alloy A is not supplied to the forbidden zone 318. In this way, it is possible to circulate the cooling water to cool one of the cooling zones down while producing the foil strip S in the other cooling zone, and thereby to produce the foil strip S having a large sheet thickness almost continuously in an industrial scale.

Moreover, in this embodiment as well, it is preferable to set the width of each of the cooling zones 313a and 313b equal to

1.5 times or more of the width of the foil strip S, which is intended to be produced, as in the case of the above-mentioned third embodiment. In this way, the heat transmitted from the molten alloy A to the cooling zones 313a and 313b is also spread in the width direction and the amount of heat discharged to the cooling water for each round of the cooling roll is increased.

On the other hand, the forbidden zone 318 interposed between the cooling zones is provided in order to equalize 10 temperature distribution in the width direction inside the cooling zones caused by alternate casting by suppressing the heat transfer between the cooling zones, and thereby to minimize an influence on the formed amorphous foil strip. It is preferable that the material of the forbidden zone 318 have 15 lower thermal conductivity than the material of the cooling zones. However, the same thermal conductivity is also acceptable. If the material of the forbidden zone 318 is the same as the material of the cooling zones, the forbidden zone 318 means a thick wall portion of the cooling roll interposed 20 between the two cooling zones where the outer circumferential surface of the cooling zone does not contact the molten alloy.

When the thermal conductivity of the forbidden zone 318 is 25 equivalent to the thermal conductivity of the cooling zones, it is preferable to set the width of the forbidden zone 318 as large as possible. In the case of the same thermal conductivity, it is preferable to set the width of the forbidden zone 318 at 30 least equal to or above  $1/3$  of the width of the amorphous alloy foil strip S. As shown in FIG. 22, if the width f of the forbidden zone falls below  $1/3$  of the width c of the foil strip S, the sheet 35 thickness of the formed amorphous alloy foil strip is inclined in the width direction. Here, in FIG. 22, sheet thickness deviation is percentage of a difference  $|t_1 - t_2|$  between sheet thicknesses  $t_1$  and  $t_2$  on both width ends of the foil strip relative to 40 an average  $t_o$  of the sheet thicknesses in the width direction. Moreover, FIG. 22 shows a case where the width c of the foil strip is equal to 150 mm, in which the sheet thickness deviation is suddenly increased if the width f of the forbidden zone becomes equal to or below 50 mm, i.e., equal to or below  $1/3$  45 of the width c of the foil strip. Here, measurement of the sheet thicknesses is carried out by use of a micrometer, which represents an average of values measured in regions near both of width ends of the foil strip each having an area of  $1 \text{ cm}^2$ . Occurrence of the sheet thickness deviation on the foil strip is not favorable because problems such as reduction in the space factor of a core or winding failures in a core winding process are caused.

Next, effects of this embodiment will be described.

In this embodiment, the cooling roll 313 of the production apparatus 301 for an amorphous alloy foil strip is provided with the two cooling zones 313a and 313b and the foil strips S are cast by alternately using these zones. In this way, the single cooling zone repeats casting and cooling down, whereby it is possible to set the roll temperature equal to or 55 below the predetermined value. As a result, it is possible to produce the amorphous alloy foil strip having a large sheet thickness in an industrial scale. The amorphous alloy foil strip is applicable to a power transformer or a core of a motor, for example, and is also applicable to a magnetic shield material.

Moreover, in this embodiment, the cooling zone 313a and the cooling zone 313b are disposed distant from each other, and the forbidden zone 318 having the predetermined width is interposed between the cooling zones, and no molten alloy is supplied to the forbidden zone 318. Accordingly, it is possible 60 to render the cooling zones thermally independent of each other. In this way, it is possible to produce the thick foil strips at high productivity while ensuring the cooling rate, to sup-

press inclination of the temperature of one of the cooling zones in the width direction due to presence of the other cooling zone, and thereby to prevent the foil strips from causing the sheet thickness deviation.

Operations and effects of this embodiment other than those mentioned above are similar to the above-described third embodiment. For example, since the multiple-sift nozzle is also used as the nozzle 315 in this embodiment, it is possible to equalize the sheet thickness of the foil strips S and to reduce occurrence of pin holes. Moreover, since this embodiment also employs the cooling zones having a large wall thickness, it is possible to eliminate various problems attributable to the uneven thermal deformation of the roll, which may occur frequently in the case of using the conventional thin wall roll. For example, local embrittlement or fluctuation in magnetic characteristics of the foil strips S due to uneven cooling of the foil strips or the like does not occur.

Hereinabove, the invention is described with reference to embodiments and variations. However, the invention is not limited to these embodiments and variations. For example, the invention also encompasses addition, deletion or design changes of constituents, or addition, deletion or condition changes of processes which may be carried out as appropriate by those skilled in the art as the scope of the invention as long as such actions meet the gist of the invention. Moreover, it is also possible to carry out a combination of any of the respective embodiments and the respective variations described above.

For example, in the above-described first and second embodiments, multiple crucibles may be provided corresponding to the number of cooling rolls and sequentially supplied with a molten alloy from different pouring units, one production apparatus may be provided with three or more cooling rolls, or one crucible may be provided with multiple openings to perform pouring on the multiple cooling rolls sequentially. In addition, in the above-described third and fourth embodiments, one cooling roll may be provided with three or more cooling zones. Alternatively, the scope of the invention also includes an apparatus and a method in which a cooling roll including multiple cooling zones is combined with a cooling roll including a single cooling zone, and the molten alloy is sequentially supplied to these three or more cooling zones. By increasing the cooling zones, it is possible to increase the upper limit sheet thickness of a producible foil strip. While the conventional cooling roll with the single cooling zone is capable of achieving the upper limit sheet thickness of 25  $\mu\text{m}$ , it is possible to form thick amorphous alloy foil strips, almost continuously, specifically, as thick as 50  $\mu\text{m}$  by using two cooling zones, 75  $\mu\text{m}$  by using three cooling zones, and 100  $\mu\text{m}$  by using four cooling zones. The molten metal supplying unit can also employ a tundish provided with multiple nozzles that face the outer circumferential surfaces of the cool zones.

#### [Industrial Applicability]

According to the invention, it is possible to provide an apparatus for producing an amorphous alloy foil strip and a method for producing an amorphous alloy foil strip, which

are capable of producing an amorphous alloy foil strip having a large sheet thickness in an industrial scale.

The invention claimed is:

1. An apparatus for producing an amorphous alloy foil strip, comprising:

a first cooling roll;

a second cooling roll;

a driving unit situated between the first and second cooling rolls and configured to rotate the first and second cooling rolls by rotating shaft members connected to opposite sides of the driving unit; and

a supply unit configured to supply a molten alloy sequentially to an outer circumferential surface of the first cooling roll and an outer circumferential surface of the second cooling roll,

the supply unit including:

a crucible for retaining the molten alloy;

a nozzle for ejecting the molten alloy in the crucible to outside of the crucible, and being fitted to a lower end of the crucible; and

a moving unit extending in a direction from the first cooling roll toward the second cooling roll,

the crucible being guided by the moving unit and being movable between a position where the molten alloy can be ejected to an outer circumferential surface of the first cooling roll, and a position where the molten alloy can be ejected to an outer circumferential surface of the second cooling roll.

2. The apparatus for producing an amorphous alloy foil strip according to claim 1, wherein

the first and second cooling rolls are water-cooled rolls in which cooling water is circulated inside.

3. The apparatus for producing an amorphous alloy foil strip according to claim 2, wherein

each of the first and second cooling rolls is hollow and includes an opening in a central part on one side surface of each of the first and second cooling rolls, the cooling water is supplied through the opening, and each of the cooling rolls is rotatably supported at another side surface of each of the first and second cooling rolls.

4. The apparatus for producing an amorphous alloy foil strip according to claim 2, further comprising:

a unit configured to cool the cooling water down.

5. The apparatus for producing an amorphous alloy foil strip according to claim 1, wherein

a wall thickness of each of the first and second cooling rolls is equal to or above 25 mm.

6. The apparatus for producing an amorphous alloy foil strip according to claim 1, wherein

a diameter of each of the first and second cooling rolls is in a range from 0.4 to 2.0 meters, and

a width of the first cooling roll is 1.5 times or more of a width of an amorphous alloy foil strip to be produced.

7. The apparatus for producing an amorphous alloy foil strip according to claim 1, wherein

the nozzle having a plurality of slits arranged in a circumferential direction of the cooling rolls.